

# UNITED STATES PATENT OFFICE.

MORGAN W. BROWN, OF BROOKLYN, NEW YORK.

## ART OF ORNAMENTING THE SURFACES OF BOXES, PACKAGES, &c.

SPECIFICATION forming part of Letters Patent No. 240,228, dated April 19, 1881.

Application filed February 17, 1880.

*To all whom it may concern:*

Be it known that I, MORGAN W. BROWN, of Brooklyn, Kings county, New York, have invented an Improvement in Process for Ornamenting and Decorating Purposes, of which the following is a specification.

The nature of the present invention consists in ornamenting and decorating surfaces by applying to the same transparent or pellucid gelatine or isinglass, either plain, colored, or variegated, in part or wholly, over or above a surface formed of tin or other metallic foils, previously roughened, corrugated, or wrinkled, the object of the invention being to render the surface so treated, or to which the foil and gelatine or isinglass have been applied, more attractive, and to give to it a sparkling appearance.

To enable those skilled in the arts to make and use my invention, I will describe the manner of carrying out the same.

I first take the tin or other metallic foil and break or press the surface of it into a rough, uneven, or corrugated shape. The foil in this condition is then affixed to or upon the surface to be ornamented or decorated. I then place or affix over the surface of corrugated or roughened foil a sheet of gelatine or isinglass,

the result being, as before stated, to render the surface decorated attractive to the eye, a 30 sparkling appearance being produced by the light that passes through the gelatine or isinglass and is reflected by the corrugations of the foil.

It will be seen that if plain gelatine or isinglass be employed foils of different colors can be employed advantageously, greatly increasing the effect sought to be produced, or that a like result can be arrived at by the employment of ordinary tin-foil used in connection 40 with colored or partly-colored sheets of gelatine or isinglass.

Having now set forth my invention, what I claim as new is—

The within-described process for ornamenting or decorating surfaces, which consists in affixing to the surface a body of roughened or corrugated tin or other metallic foil, and then placing over the same a sheet of plain-colored or partly-colored gelatine or isinglass, substantially as and for the purpose specified.

MORGAN W. BROWN.

Witnesses:

PETER C. PROVOST,  
DAVID B. PROVOST.